# EUROPEAN PATENT SPECIFICATION

(11) **EP 3 814 563 B1**
(45) Date of publication and mention of the grant of the patent: **16.10.2024**
(21) Application number: 19732422.1
(22) Date of filing: 14.06.2019
(51) Int. Cl.: D02G 3/32, D02G 3/44

(54) **FIRE-RESISTANT CABLED YARN AND TEXTILE**
FEUERBESTÄNDIGES VERDRILLTES GARN UND TEXTIL
FIL CÂBLÉ RÉSISTANT AU FEU ET TEXTILE

(30) Priority: 29.06.2018 GB 201810691
(43) Date of publication of application: 05.05.2021
(73) Proprietor: Arville Textiles Limited, Wetherby, Yorkshire LS22 7DQ (GB)
(72) Inventor: BEADLE, Robert, Yorkshire BD10 0AJ (GB); HULL, Nigel, Leeds Yorkshire LS22 7UR (GB)
(74) Representative: Sewell, Adrian David
(86) International application number: PCT/GB2019/051651
(87) International publication number: WO 2020/002873

(56) References cited:
- WO-A1-2014/018221
- WO-A1-2016/010659
- WO-A2-2008/097356
- JP-A- 2014 208 930
- US-A- 5 694 981

## Description

The present invention relates to fire resistant textile materials and to garments manufactured from such materials. In particular, but not exclusively, the present invention relates to articles of fire resistant clothing for use by fire fighters, military personnel and police officers, or the like, and to textiles for manufacturing such clothing.

Clothing for protection against heat and flame must pass minimum performance requirements for flame, radiant heat, heat resistance, tensile and tear strength, and penetration by water and liquid chemicals. The assembled garments, which typically include a pair of trousers/salopettes and a jacket, must protect the wearer from radiant and thermal exposure, and unexpected flashover conditions, whilst still maintaining an adequate level of dexterity and comfort.

As described in WO2015/008030, it is known to reduce second and third degree burns to a wearer by ensuring the barrier of protective clothing located between the heat source and the wearer's skin remains intact during exposure to heat and flame whilst ensuring an air gap exists between the skin and the heat source. It is also known to provide a single woven layer of fire-resistant textile material which utilises the strength characteristics of meta-aramid fibres in a warp yarn and the moisture management properties of wool in a blended wool and cellulose weft yarn for direct contact against a wearer's skin. Other known methods are described in JP2014 208930, WO2016/010659 and WO2008/097356.

However, conventional fire-resistant textile materials are relatively heavy, allow for limited movement, and do not sufficiently and efficiently move moisture in the form of sweat away from the skin which can otherwise result in steam/scald burns. Furthermore, the demand for fire-resistant garments which are lighter in terms of weight and with improved comfort, breathability and moisture management is ever increasing.

It is an aim of certain embodiments of the present invention to provide a fire-resistant textile material which is lightweight, breathable, strong, durable and comfortable.

According to a first aspect of the present invention there is provided a cabled yarn according to claim 1.

Optionally, the cellulose fibres comprise a fire-retardant viscose fibre.

According to a second aspect of the present invention there is provided a fire-resistant textile material comprising a cabled yarn according to the first aspect of the present invention.

Optionally, the textile material comprises the yarn in both warp and weft directions.

Optionally, the warp and weft yarns define a twill weave.

According to a third aspect of the present invention there is provided a garment comprising a material according to the second aspect of the present invention.

According to a fourth aspect of the present invention there is provided a method of manufacturing a cabled yarn according to claim 7.

According to a fifth aspect of the present invention there is provided a method of manufacturing a fire-resistant textile material, comprising:
weaving yarn according to the first aspect of the present invention in both warp and weft directions.

Optionally, the weave is a twill weave.

### Description of the Drawings

Certain embodiments of the present invention will now be described with reference to the accompanying drawings in which:
Figure 1 illustrates a 'cabled' three-ply yarn according to certain embodiments of the present invention.

### Detailed Description

According to certain embodiments of the present invention, a single ply yarn includes a blend of paraphenylene isophthalamide (meta-aramid) fibres, cellulose-based fibres, wool fibres, and polyparaphenylene terephthalamide (para-aramid) fibres. Aptly, the meta-aramid fibre is Nomex^{™} and the para-aramid fibre is Kevlar^{™}. Aptly, the cellulose-based fibre is Lenzing^{™} FR.

As illustrated in Figure 1, two of these single ply yarns 100 are twisted together with a third yarn of substantially elastic fibre 110 to form a 'cabled' three-ply yarn 200. The elastic fibre 110 is located centrally with the single ply yarns 100 twisted therearound to provide effective cover and protection to the elastic fibre. The centrally located elastic fibre yarn 110 comprises Elastolefin^{™} which is a fibre composed of at least 95% (by weight) of macromolecules partially crosslinked, made of ethylene and at least one other olefin. When stretched by up to 50% of its original length, it recovers rapidly to its original length.

The composition (by weight) of the fibre components of the cabled yarn 200 is:
- around 33% Lenzing^{™} FR;
- around 33% wool;
- around 23% meta-aramid (Nomex^{™});
- around 7% Elastolefin^{™} XLA; and
- around 4% para-aramid (Kevlar^{™}).

Aptly, the Lenzing^{™} FR fibre has a linear mass density of around 2.2 dtex and comprises a fire-retardant viscose fibre. The Lenzing^{™} fibres offer moisture management with its efficient moisture wicking and transportation properties when worn next to the skin of a wearer in combination with its quick drying and comfort properties.

The wool fibres have a thickness of between around 15.5-29.5 µm, and aptly around 19.5 µm which has been found to be optimum in terms of efficient and effective transportation of moisture from the skin and across adjacent fibres. The wool fibres are treated to be shrink resistant. The wool fibres are hygroscopic such that they can hold up to a third of their own weight in moisture without feeling wet thereby helping to wick away sweat whilst enhancing comfort. The hygroscopic properties of the wool fibres also help to regulate temperature and humidity, creating a buffer area (i.e. holds moisture without feeling wet), enhancing comfort. Furthermore, the chemical building blocks of wool, i.e. amino acids, are hydrophilic (water-liking) such that they attract and absorb water molecules into the chemical structure of the fibre. Water binds within the wool structure through the action of hydrogen bonds in a process known as absorption. Wool is inherently antimicrobial and antistatic which enhances comfort and protection. Wool has a helical configuration in the centre of the fibre which acts like a shock absorbing spring under compression which further enhances comfort for a wearer.

Nomex^{™} yarn is typically available in three types based on the linear mass density (2.2 dtex, 1.7dtex and 1.4dtex). Aptly, a 1.4dtex Nomex^{™} yarn is used as it offers desirable comfort and flexibility in view of its fineness.

The XLA fibres have a linear mass density of around 117 dtex. XLA is particularly fire-resistant, robust and accommodates high levels of activity and movement to provide enhanced comfort for many different applications.

Kevlar^{™} is a preferred para-aramid fibre in view of its high strength, chemical resistance, excellent durability and thermal stability. The para-aramid fibre is around 1.7 dtex / 50 mm staple length as it is aptly a spun yarn.

The cabled three-ply yarn 200 is aptly used to provide a textile according to certain embodiments of the present invention which may be used for a fire-resistant garment, e.g. a fire fighter's jacket. The weave is aptly a 2x2 twill weave but other suitable weave patterns may be used such as a plain weave, 2x1, 3x1, 4x1 or 2x2 twill weaves, ripstop or hopsack weaves, satin, or sateen weaves, or the like. A 2x2 twill weave is desirable because it allows movement when shrinking down the fabric for stretch due to float size. A twill weave also desirably provides a tighter, denser construction which enhances the dimensional stability and increases durability after multiple washing. The cabled three-ply yarn 200 is in both warp and weft directions to desirably provide stretch in all four directions (horizontally, vertically, and diagonally) thereby providing optimal comfort to a wearer of a garment made from the textile.

The textile is scoured, heat sett and pressed to provide a smooth and comfortable garment. Such a garment may include trousers, salopettes, jackets, overalls, T-shirts, facemasks, falsehoods, or the like. Applications for such a garment may include tackling wild land fires, electric arc protection, petrochemical applications, search & rescue, forestry, police violent situation/riot protection, military, or the like.

In accordance with certain embodiments of the present invention, the final yarn may comprise more than three plies, e.g. four or more plied yarns twisted around a centrally located and substantially elastic yarn. For example, the final yarn may include antistatic fibres. A multi-ply yarn is often known as a cabled or hammer yarn.

A key technical advantage of utilising these yarns in personal protective equipment (PPE) applications, particularly fire-resistant garments, is to provide a stretch material to maximise comfort whilst maintaining strength and integrity and offering sufficient protection against flame and heat. The aramid fibres offer strength and robustness to withstand wear during use and to hold the material together during flaming/extreme heat exposure, whilst the XLA fibres provide desirable stretch. The 'maypole' construction of the cabled yarn desirably protects the centrally located XLA yarn against flame, heat, UV, or the like.

## Claims

1. A cabled yarn (200) comprising:
at least two single plied yarns (100) each comprising meta-aramid fibres, para-aramid fibres, cellulose-based fibres, and wool fibres, twisted around a centrally located yarn (110) comprising an Elastolefin fibre, wherein the cabled yarn (200) comprises by weight around 23% meta-aramid fibres, around 4% para-aramid fibres, around 33% cellulose-based fibres, around 33% wool fibres, and around 7% Elastolefin fibres, and wherein the wool fibres have a thickness of around 15.5µm to around 29.5µm.

2. The yarn according to claim 1, wherein the cellulose fibres comprise a fire-retardant viscose fibre.

3. A fire-resistant textile material comprising a cabled yarn (200) according to any preceding claim.

4. The textile material according to claim 3, comprising the yarn in both warp and weft directions.

5. The textile material according to claim 4, wherein the warp and weft yarns define a twill weave.

6. A garment comprising a material according to any of claims 3 to 5.

7. A method of manufacturing a cabled yarn (200), comprising:
twisting at least two single plied yarns (100) each comprising meta-aramid fibres, para-aramid fibres, cellulose-based fibres, and wool fibres, around a centrally located yarn (110) comprising an Elastolefin fibre, wherein the cabled yarn (200) comprises by weight around 23% meta-aramid fibres, around 4% para-aramid fibres, around 33% cellulose-based fibres, around 33% wool fibres, and around 7% Elastolefin fibres, and wherein the wool fibres have a thickness of around 15.5µm to around 29.5µm.

8. A method of manufacturing a fire-resistant textile material, comprising:
weaving yarn according to any of claims 1 and 2 in both warp and weft directions.

9. The method according to claim 8, wherein the weave is a twill weave.

## Patentansprüche

1. Verdrilltes Garn (200), umfassend:
Mindestens zwei einfach gezwirnte Garne (100), wobei jedes Meta-Aramidfasern, Para-Aramid-Fasern, Fasern auf Zellulosebasis und Wollfasern umfasst, die um ein mittig positioniertes Garn (110) verdrillt sind, das eine Elastolefin-Faser beinhaltet, wobei das verdrillte Garn (200) gewichtsmäßig etwa 23 % Meta-Aramidfasern, etwa 4 % Para-Aramid-Fasern, etwa 33 % Fasern auf Zellulosebasis, etwa 33 % Wollfasern und etwa 7 % Elastolefin-Fasern umfasst, und wobei die Wollfasern eine Dicke von etwa 15,5 µm bis etwa 29,5 µm aufweisen.

2. Garn nach Anspruch 1, wobei die Fasern auf Zellulosebasis eine feuerbeständige Viskosefaser umfassen.

3. Feuerbeständiges textiles Material, das ein verdrilltes Garn (200) nach irgendeinem vorhergehenden Anspruch umfasst.

4. Textiles Material nach Anspruch 3, welches das Garn in sowohl in Kett- als auch in Schussrichtungen umfasst.

5. Textiles Material nach Anspruch 4, wobei die Kett- und Schussgarne eine Köperbindung definieren.

6. Kleidungsstück, das ein Material nach irgendeinem der Ansprüche 3 bis 5 umfasst.

7. Verfahren zur Herstellung eines verdrillten Garns (200), umfassend:
Zwirnen von mindestens zwei einfach gezwirnten Garnen (100), die jeweils Meta-Aramidfasern, Para-Aramid-Fasern, Fasern auf Zellulosebasis und Wollfasern umfassen, um ein mittig positioniertes Garn (110), das eine Elastolefin-Faser umfasst, wobei das verdrillte Garn (200) gewichtsmäßig etwa 23 % Meta-Aramidfasern, etwa 4 % Para-Aramid-Fasern, etwa 33 % Fasern auf Zellulosebasis, etwa 33 % Wollfasern und etwa 7 % Elastolefin-Fasern umfasst, und wobei die Wollfasern eine Dicke von etwa15,5 µm bis etwa 29,5 µm aufweisen.

8. Verfahren zur Herstellung eines feuerbeständigen textilen Materials, umfassend:
Weben von Garn nach irgendeinem der Ansprüche 1 und 2 in sowohl Kett- als auch Schussrichtungen.

9. Verfahren nach Anspruch 8, wobei die Webart eine Köperbindung ist.

## Revendications

1. Fil câblé (200) comprenant :
au moins deux fils retors simples (100) comprenant chacun des fibres de méta-aramide, des fibres de para-aramide, des fibres à base de cellulose, et des fibres de laine, torsadés autour d'un fil positionné centralement (110) comprenant une fibre d'élastoléfine, dans lequel le fil câblé (200) comprend, en poids, environ 23 % de fibres de méta-aramide, environ 4 % de fibres de para-aramide, environ 33 % de fibres à base de cellulose, environ 33 % de fibres de laine, et environ 7 % de fibres d'élastoléfine, et dans lequel les fibres de laine ont une épaisseur d'environ 15,5 µm à environ 29,5 µm.

2. Fil selon la revendication 1, dans lequel les fibres de cellulose comprennent une fibre de viscose ignifugeante.

3. Matériau textile résistant au feu comprenant un fil câblé (200) selon l'une quelconque des revendications précédentes.

4. Matériau textile selon la revendication 3, comprenant le fil dans les sens à la fois chaîne et trame.

5. Matériau textile selon la revendication 4, dans lequel les fils chaîne et trame définissent une armure sergée.

6. Vêtement comprenant un matériau selon l'une quelconque des revendications 3 à 5.

7. Procédé de fabrication d'un fil câblé (200), comprenant :
le retordage d'au moins deux fils retors simples (100) comprenant chacun des fibres de méta-aramide, des fibres de para-aramide, des fibres à base de cellulose, et des fibres de laine, autour d'un fil positionné centralement (110) comprenant une fibre d'élastoléfine, dans lequel le fil câblé (200) comprend, en poids, environ 23 % de fibres de méta-aramide, environ 4 % de fibres de para-aramide, environ 33 % de fibres à base de cellulose, environ 33 % de fibres de laine, et environ 7 % de fibres d'élastoléfine, et dans lequel les fibres de laine ont une épaisseur d'environ 15,5 µm à environ 29,5 µm.

8. Procédé de fabrication d'un matériau textile résistant au feu, comprenant :
le tissage d'un fil selon l'une quelconque des revendications 1 et 2 dans les sens à la fois chaîne et trame.

9. Procédé selon la revendication 8, dans lequel l'armure est une armure sergée.
